

## UNITED STATES PATENT OFFICE

HERBERT HÖNEL, OF VIENNA, AUSTRIA, ASSIGNOR TO BECK, KOLLER & COMPANY, INC.,  
OF DETROIT, MICHIGAN, A CORPORATION OF DELAWARE

MIXED ESTER COMPOSITION AND PROCESS OF MAKING THE SAME

No Drawing.

Application filed June 6, 1930. Serial No. 459,613.

The invention relates to the production of mixed ester compositions and to the process of making the same.

This application is a continuation in part of my application Serial No. 454,186, filed May 20, 1930, which in turn is a continuation in part of my prior application Serial No. 362,460, filed May 11, 1929, now Patent No. 1,800,296, dated April 24, 1931.

It is known to combine natural resins with condensation products obtained from phenols with aldehydes and the like, by employing elevated temperatures. Products of special technical and economic importance are apparently created by reacting fresh acid rosins (of conifers) together with relatively small amounts of low molecular phenol alcohols. As known, the latter are condensation products obtained by means of alkali from phenols and formaldehyde and are rendered insoluble when heated alone. When proper proportions and conditions are employed the resulting products are clear and soluble in common solvents without residue. Their hardness and melting point are much higher than that of the rosin itself, but their acid value is still of corresponding value to that of the rosin itself, and it has been suggested to esterify them with alcoholic bodies as has been practiced a long time previously with acid rosins themselves. Such esterified products also possess improved properties as compared with the common rosin esters themselves, such as increased toughness, hardness and melting point.

But it is a disadvantage of these products that they are not compatible with nitrocellulose, even if very small amounts only of phenol alcohols have been employed.

I have formed new and very useful products by esterifying said reaction products of the acid rosin and phenol alcohols and a relatively low molecular carboxylic acid with a polyhydric alcohol. Doubtless mixed esters of the polyhydric alcohol result from

this procedure. The relative increase of the ester groups by introducing such relatively low molecular carboxylic acid groups in the molecule apparently causes the compatibility with nitrocellulose. The employment of acids of the aromatic series has been found to be superior to the use of acids of the aliphatic series. Furthermore it is evident that polybasic acids which still further increase the relative amount of ester groups therefore may be used advantageously. The resulting esterlike products are also particularly tough and hard. The quantity of such acids employed must be limited, as otherwise insoluble masses might result.

Furthermore, I have advantageously employed these new resins in combination with drying vegetable oils to make a varnish. The combination with fatty oils mostly succeeds only at higher temperatures, i. e. 240-280° C. This probably takes place by means of re-esterifications. In accordance with this conception the combination takes place more readily when the fatty oils are added before the esterification is carried out. In this case soluble products result even if larger amounts of the polybasic acids are used. The combination with the fatty oils takes place more readily when the fatty oils are partly substituted by their fatty acids and the corresponding amount of glycerine. Of course, theoretically the whole amount of the oil may be substituted by its fatty acids, but this would be uneconomical. The resinlike solid products obtained according to my process are soluble in the usual mixtures of solvents for cellulose esters and generally also in benzol hydrocarbons, while their solubility in petroleum hydrocarbons is mostly unsatisfactory. Products combined with fatty oils are mostly soluble in the cheap petroleum hydrocarbons, or at least in mixtures of these with benzol hydrocarbons. The solutions themselves can be employed in the same way as common oil varnishes with driers, but they

produce a still tougher and harder film. These products combined with fatty oils are also very adaptable as ingredients in nitrocellulose lacquers in suitable solvents, as are the above described solid resins themselves. A simultaneous addition of plasticizers is superfluous when such products combined with fatty oils are employed. For such purposes products are very advantageous which are combined with castor oil. Castor oil readily enters into the chemical composition and allows the formation of very pale products.

The term "low molecular" as used in the specification and claims as applied to acids employed is intended to distinguish such acids from the relatively high molecular natural resin acids.

A few examples may explain my process:  
**Example 1.**—A liquid phenol alcohol is formed from 150 parts of a technical mixture of m-p-cresol and 180 parts of formaldehyde (40 volume %) by means of alkali and then introduced into 1000 parts of melted French rosin WG. The temperature of the melt is raised to a maximum of 210° C. A clear resin is obtained which has a melting point of about 100 to 110° C. and an acid number of about 140. 300 parts of benzoic acid and 200 parts of glycerine (95%) are added and the temperature raised under continued stirring until a uniform reacting mass is obtained. Finally the esterification is carried out at 270° C. The resulting resin has a rather low melting point, but is very tough and has very good adhesion. It is soluble in benzol hydrocarbons and the usual mixtures of solvents for nitrocellulose and produces a clear film in connection with nitrocellulose in all proportions, showing many desirable properties.

**Example 2.**—100 parts of American rosin WW are reacted with a liquid phenol alcohol obtained from 12 parts of USP cresol and 135 parts of formaldehyde (40 volume %) as described in Example 1. The reacting product is esterified simultaneously with 20 parts of phthalic anhydride and 20 parts of glycerine. The resulting product has a melting point of 108-120° C. and an acid number of about 20 and is very hard and tough. Its color is light reddish brown. The color can be considerably improved, when phthalic anhydride and glycerine (or at least part of the latter) are first heated alone until a sticky reaction product is formed which is practically free from phthalic anhydride and this reaction product is then combined with that resulting from the rosin and the phenol alcohol. The reaction product or phthalic anhydride and glycerine may show an acid number of 160 to 230, and is to be considered as a partial ester which still contains free carboxylic and alcoholic groups. The other properties are equal to those obtained by the

products resulting from the first method. They are very adaptable both for use in nitro lacquers and in oil varnishes. In the latter case, they must be heated with the drying oil or a part of it to about 260-280° C. to get a clear solution.

It should be mentioned that an esterlike product which is obtained from 20 parts of phthalic anhydride and 20 parts of glycerine and 100 parts of American rosin itself, (i. e. the same proportions employed as in Example 2, but without employing the phenol alcohol) lacks by far that hardness and toughness and has a melting point of only 66-74° C., i. e. like the plain glycerine rosin ester.

**Example 3.**—The reaction products from 100 parts of rosin and phenol alcohol as in Example 2, 12 parts of succinic acid, 4 parts of butyric acid and 20 parts of glycerine are esterified together under conditions similar to those described in the other examples. In the first part of the esterification it must be taken care that the relatively low boiling butyric acids does not leave the reacting mass. The very pale, hard and tough final product is highly adaptable for use in nitrocellulose lacquers.

**Example 4.**—A condensation product is prepared as follows: To 100 parts of technical meta cresol which usually contains about 60% meta cresol and 40% para cresol are introduced carefully and under cooling 75 parts of sulphuryl chloride. Under splitting off of SO<sub>2</sub> and HCl merely the m-cresol will be chlorinated in the p-position, while the p-cresol will remain untouched. After washing and neutralizing the reaction product a condensation product is formed with 140 parts of formaldehyde (40 volume %) by means of alkali. The condensation product, which is a reddish oily and crystalline mass, is caused to react with 600 parts of Spanish crystal rosin in a manner as disclosed in the above examples. Afterwards 400 parts of phthalic anhydride, 280 parts of glycerine and 100 parts of linseed oil fatty acids are added and heated under stirring to about 200° C. When the reacting mass has become clear and uniform, 300 parts of linseed oil and 150 parts of China wood oil are slowly added. Then the temperature is raised to 260-270° C. and held until the acid number is sufficiently low and the mass shows the desired consistency. It is a very satisfactory base for varnishes and can also be incorporated in nitrocellulose lacquers in every proportion.

It has been found that by the use of phenols which are substituted in the p-position, final products are formed of satisfactory light proofness.

**Example 5.**—In Example 4 the fatty acids and 13 parts of glycerine, the linseed oil and the China oil are substituted by 450 parts

of castor oil. The glycerine and the phthalic anhydride are first heated alone as described in Example 2 until the mass has an acid number of about 220. For the rest the same conditions are employed. The resulting product is very pale and tough and can be used as a base for quick-drying enamels with or without addition of nitrocellulose.

It will be understood that the above description and specific examples are given by way of illustration rather than by way of limitation and known equivalents of the substances set forth may be substituted for those given by way of illustration. Thus, while in the examples set forth above, only vegetable oils are mentioned, as illustrative of the fatty oils, it is contemplated that other fatty oils may be used, as for example, fish oils. Likewise, other substitutes for the other original or starting substances may be employed.

By relatively low molecular carboxylic acids I have reference to carboxylic acids such as butyric, benzoic, succinic, maleic, adipic, phthalic, camphoric, and citric which are crystalline in character as distinguished from relatively high molecular monobasic and polybasic acids such as natural resinous acids or fatty acids of either unaltered or polymerized natural glycerides having more or less colloidal properties as distinguished from crystalline.

What I claim is:

1. A process which comprises esterifying the acid product obtained by the reaction of a fresh natural resin and phenol alcohol, by combining with such acid product a relatively low molecular carboxylic acid and polyhydric alcohol.

2. As a new composition of matter, an esterlike reaction product of (1) a polyhydric alcohol combined with (2) the reaction product of a fresh natural resin acid and (3) phenol alcohol and a relatively low molecular carboxylic acid.

3. A product according to claim 2 which is combined with a fatty oil.

4. A product according to claim 2 which is combined with a fatty oil of the drying type.

5. A mixed ester of a polyhydric alcohol, which ester contains as acid groups (1) the reaction product of a natural resin acid with a phenol alcohol and (2) a relatively low molecular carboxylic acid and (3) the acids of a fatty oil.

6. A new composition of matter formed by the reaction of (1) a natural resin acid, (2) a phenol alcohol, (3) at least one member of a group consisting of relatively low molecular polybasic carboxylic acids and anhydrides, and (4) a polyhydric alcohol.

7. A process of producing artificial masses which comprises reacting (1) a natural resin acid, (2) a phenol alcohol, (3) at least one

member of a group consisting of relatively low molecular polybasic carboxylic acids and anhydrides, and (4) a polyhydric alcohol.

8. A new composition of matter formed by the reaction of (1) a natural resin acid, (2) a phenol alcohol, (3) phthalic anhydride, and (4) glycerine.

9. A process of producing artificial masses which comprises reacting (1) a natural resin acid, (2) a phenol alcohol, (3) phthalic anhydride, and (4) glycerine.

In testimony whereof I affix my signature.

HERBERT HÖNEL.

80

85

90

95

100

105

110

115

120

125

130